

## UNITED STATES PATENT OFFICE

2,564,634

## LUBRICANT CONTAINING HYDROABIETYL ESTERS

Leslie C. Beard, Jr., New York, N. Y., and Ralph V. White, Pitman, N. J., assignors to Socony-Vacuum Oil Company, Incorporated, a corporation of New York

No Drawing. Application April 8, 1949,  
Serial No. 86,382

9 Claims. (Cl. 252—48.4)

1

The present invention relates to improved lubricants, and more particularly, to improved lubricants comprising mineral oil containing esters of dehydro-, dihydro-, and tetrahydroabietyl alcohol which alcohols are obtained in admixture, known to the trade as hydroabietyl alcohol. The mixture available in industry as hydroabietyl alcohol is composed of 13-15 per cent of a non-alcohol fraction and the balance is about 15 per cent dehydroabietyl alcohol, 40 per cent dihydroabietyl alcohol and 45 per cent tetrahydroabietyl alcohol. It will be understood that the distribution of the alcohols averages that given hereinbefore but will vary from batch to batch.

The physical properties and composition of hydroabietyl alcohol are as follows:

|                                                         |                  |
|---------------------------------------------------------|------------------|
| Hydroxyl value.....                                     | 5.0-5.1 per cent |
| Hydroabietyl alcohol.....                               | 85-87 per cent   |
| Saponification number (diethyl-<br>ene glycol No.)..... | 5-14             |
| Acid number.....                                        | 0.1-0.4          |
| Methoxyl value.....                                     | 0.5-1.2          |
| Unsaturation, weight per cent:                          |                  |
| By hydrogen absorption.....                             | 0.60-0.75        |
| By bromine number.....                                  | 12-30            |
| Color (50-mm. tube) Lovibond.....                       | 0.5 amber        |
| U. S. Rosin Standard.....                               | Z <sub>7</sub>   |
| Softening point (drop method).....                      | 33° C.           |
| Specific gravity at 20°/20° C.....                      | 1.007-1.008      |
| Refractive index at 20° C.....                          | 1.528            |
| Flash point (C. O. C.).....                             | 185-195° C.      |
| Flame point (C. O. C.).....                             | 217-220° C.      |

It has been said that the chemical reactions of hydroabietyl alcohol are typical of a primary monohydric alcohol plus what might be expected from the residual unsaturation in the ring structure. Nevertheless, it has been found that as an additive to mineral oil to produce a compounded mineral oil for use as a gear lubricant or a cutting oil or a turbine oil, the similarity between esters of hydroabietyl alcohol and esters of a primary monohydric aliphatic alcohol ceases to exist. It is true that hydroabietyl alcohol reacts with mono- and dicarboxylic acids to produce esters but the similarity between hydroabietyl alcohol and oleyl alcohol, for example, ceases at that point. However, before discussing the marked difference between esters of hydroabietyl alcohol and esters of alcohols such as oleyl alcohol, it is desirable to emphasize the structure of the alcohols present in hydroabietyl alcohol. It also is to be noted that the non-alcohol portion of hydroabietyl alcohol varies with the saponification number but will average 3-8 per cent of esters which can be considered as methyl esters

2

of hydrogenated rosin and the remainder 7-12 per cent is similar to the hydrocarbon fractions occurring in hydrogenated rosin. Thus, the product, esters of hydroabietyl alcohol, may give the improved results to be discussed hereinafter because of the structure of the alcohol, because of the degree of unsaturation of the major portion of the alcohol fraction or for other reasons at present unknown.

10 The three alcohols present in hydroabietyl alcohol have the following structures:



30 It will be noted that in each alcohol the hydroxyl group is attached to the nucleus through a methylene, CH<sub>2</sub>, group. It also will be noted that an isopropyl group and two methyl groups are attached to the nucleus. Although 45 per cent of the abietyl alcohols present is a saturated alcohol the balance is alcohols of two degrees of unsaturation. Consequently, the major portion of the alcohol portion of hydroabietyl alcohol is alcohols having one and three olefinic double bonds.

35 It has been found that esters prepared from the commercial hydroabietyl alcohol and hydroxy aliphatic polycarboxylic acids are useful as rust inhibitors in turbine oils and as extreme pressure additives in lubricants such as gear oils. Typical esters are di-hydroabietyl malate, di-hydroabietyl tartrate, tri-hydroabietyl citrate, hydroabietyl-2-ethylhexyl malate, hydroabietyl-2-ethylhexyl tartrate, di-hydroabietyl-2-ethylhexyl citrate, hydroabietyl-oleyl malate, hydroabietyl-oleyl tartrate, di-hydroabietyl-oleyl citrate, hydroabietyl dioleyl citrate, and similar esters of

hydroxy aliphatic polycarboxylic acids in which all of the carboxyl groups are esterified with hydroabietyl alcohol or in which one carboxyl group of a dicarboxylic acid is esterified with hydroabietyl alcohol and the other carboxyl group is esterified with a monohydric aliphatic saturated or unsaturated straight chain or branched chain alcohol of at least 8 carbon atoms or 1 or two carboxyl groups of a tricarboxylic acid are esterified with hydroabietyl alcohol and the others esterified by a monohydric saturated or unsaturated straight or branched chain monohydric alcohol of at least 8 carbon atoms. It is to be understood that the term hydroabietyl alcohol is used herein to designate the mixture of alcohols, esters and hydrocarbons discussed hereinbefore.

In determining the amount of hydroabietyl alcohol to be reacted with a predetermined amount of polycarboxylic acid, it is necessary to bear in mind that the presently available commercial hydroabietyl alcohol is, as pointed out hereinbefore, a mixture of alcohols, esters and hydrocarbons. Consequently, the amount of the mixture employed will be dependent upon the hydroxyl number of the available commercial hydroabietyl alcohol. One gram molecular weight of hydroabietyl alcohol contains 17 grams of the hydroxyl group. A determination of the hydroxyl number of the commercial hydroabietyl alcohol used in the preparations discussed hereinafter established that 341 grams of that commercial hydroabietyl alcohol contained 17 grams of the hydroxyl group. Therefore, for each mole of polycarboxylic acid employed in the preparation of an ester 17 grams of hydroxyl group are required for each carboxyl group to be esterified by the hydroabietyl alcohol. Consequently, when preparing dihydroabietyl malate from 0.375 mole of dl-malic acid 0.75 mole of hydroabietyl alcohol is required. Since 341 parts by weight of commercial hydroabietyl alcohol having a hydroxyl value of 5% contains 17 parts by weight of hydroxyl group, it follows that 0.375 mole of malic acid require 75% of 341 or 255.7 parts by weight of commercial hydroabietyl alcohol.

Di-hydroabietyl malate was prepared by placing 0.75 mole (255.7 g.) commercial hydroabietyl alcohol and 0.375 mole of dl-malic acid in a container provided with a thermometer, a mechanical stirrer and a reflux condenser provided with a water take-off. The mixture was heated to 130°-135° C. and digested in that temperature range for about 0.5 hour. The reflux water take-off was filled with benzene and an amount of benzene added to the reaction mixture such that the benzene refluxed while the contents of the reactor were at 130°-135° C. (Any other solvent forming an azeotropic mixture with water can be used.) After refluxing for 6 hours 93 per cent of the

water of reaction had been separated. The solvent was then removed by gradually reducing the pressure in the reactor. The solvent-free product was warmed to 130° C., and filtered to remove solids. The filtered product had a neutralization number of 13.3 indicative of neutral ester content of about 89 per cent.

Hydroabietyl-2-ethylhexyl malate was prepared in a manner similar to that employed in preparing di-hydroabietyl malate by reacting 0.5 mole of hydroabietyl alcohol, 0.5 mole 2-ethylhexanol and 0.5 mole dl-malic acid. The filtered product had a neutralization number of 19.9 indicative of a neutral ester content of about 88.6 per cent.

Hydroabietyl oleyl malate was prepared from 0.375 mole of hydroabietyl alcohol, 0.375 mole of oleyl alcohol and 0.375 mole of dl-malic acid. The filtered product had a neutralization number of 16.0 indicative of a neutral ester content of about 88 per cent.

Each of the foregoing products was subjected to the A. S. T. M. Test D665-44T. In this test, a cylindrical polished steel specimen is suspended and soaked in 300 milliliters of the test oil at 140° F., for 30 minutes. Thirty milliliters of distilled water are added then and the mixture is stirred at 1000 R. P. M. After 48 hours the steel specimen is removed and examined for evidence of rust. The oil is rated as passing when there is no evidence of rust on that part of the specimen which hangs below the oil level.

The test oil for the anti-rust tests was a blend of solvent-refined Mid-Continent residual stock with a solvent-refined Mid-Continent distillate stock. The blend has a specific gravity of 0.872, a flash point (C. O. C.) of 445° F., and Saybolt Universal viscosity of 407.7 seconds at 100° F. This oil is suitable for use in steam turbines. In addition to the esters to be tested the oil blend contained 0.2 per cent of tertiary butyl para cresol and 0.1 per cent of phenyl alpha naphthylamine. These antioxidants may be replaced by other suitable antioxidants.

The oils which were subjected to the anti-rust test were also subjected to the Emulsion Test for Lubricating Oils described in the Federal Stock Catalogue, Section IV, Part 5, Federal Specification VV-L-791b (February 19, 1942). In the test 320.13, 40 milliliters of the oil blend to be tested and 40 milliliters of emulsant are stirred for 5 minutes with a paddle at 1500 R. P. M. in a 100 milliliter graduated cylinder at 130° F. Separation of the emulsion is observed while the cylinder is maintained at 130° F. The number of minutes required for the disappearance of a continuous layer of emulsion between the oil and the emulsant is recorded.

The results of the tests described hereinbefore are recorded in Table I.

TABLE I

| Anti-rust Agent                                 | Anti-rust Agent Cone., Per Cent weight | ASTM Rust Test (D665-44T) Distilled Water | Govt. Emulsion Test @ 130° F. (Method 320.13) Minutes to break |         |
|-------------------------------------------------|----------------------------------------|-------------------------------------------|----------------------------------------------------------------|---------|
|                                                 |                                        |                                           | Distilled Water                                                | 1% NaCl |
| Di-hydroabietyl Malate                          | 0.25                                   | pass (perfect)                            | 13                                                             | 16      |
| Hydroabietyl Octyl <sup>1</sup> Malate          | 0.25                                   | do                                        | 15                                                             | 13      |
| Hydroabietyl Oleyl Malate                       | 0.25                                   | do                                        | 17                                                             | 19      |
| Base Oil (with or without oxidation inhibitors) | 0.00                                   | fail (severe rust)                        | 2                                                              | 1       |

<sup>1</sup> Octyl is 2-ethylhexyl.



where R' is a high molecular weight olefinic radical and R'' is the radical from the hydroabietyl alcohol mixture.

Thus, although the only apparent difference between the esters is the substitution of a hydroabietyl radical for one of the partially esterified dihydric alcohol radicals, the novel ester is about twice as efficient as the prior art ester-type additive.

While the tapping, threading and "drill life" tests indicate that esters having both carboxyl groups of an hydroxy aliphatic polycarboxylic acid esterified with radicals from hydroabietyl alcohol mixture are all more effective than similar esters of aliphatic alcohols, there is an advantage to the use of either mixed esters or mixtures of esters. This advantage results from the viscosity of the various esters. As is manifest after a consideration of the following tabulation of viscosities of various esters, di-hydroabietyl malate, for example, is far more viscous than the mixed esters. The high viscosity of the di-hydroabietyl esters makes it desirable to reduce the viscosity without sacrificing a disproportionate amount of the effectiveness of the hydroabietyl esters. As will be appreciated by study of the following tabulation this can be done by using mixed esters.

| Ester                             | Tanning Efficiency, Per Cent | Oster Threading Efficiency, Per Cent | Viscosity At 130° F. | SUV (sec.) At 210° F. |
|-----------------------------------|------------------------------|--------------------------------------|----------------------|-----------------------|
| Di-hydroabietyl malate            | 101                          | 101                                  | -----                | 2,641                 |
| Hydroabietyl oleyl malate         | 110                          | 102                                  | 730                  | 104                   |
| Hydroabietyl-2-ethyl-hexyl malate | 102                          | 100                                  | 1,668                | 134                   |

Consequently, for ease of manufacture and incorporation in oil blends it is preferred to employ a mixed ester of an alphahydroxy polycarboxylic acid derived from 50 mole per cent of hydroabietyl alcohol (based upon the hydroxyl number of alcohol mixture) and 50 mole per cent oleyl alcohol, i. e., from the reaction of 1 mole of hydroabietyl alcohol, 1 mole of oleyl alcohol and 1 mole of polycarboxylic acid. Fluidity of the product can be obtained by employing mixed esters of alpha-hydroxy polycarboxylic aliphatic acids in which from 50 mole per cent to 100 mole per cent hydroabietyl radical and from 1 to 50 mole per cent of an alkyl radical are present in the carbalkoxy groups (carbalkoxy being inclusive of carbocycloalkoxy). The alkyl groups are those derived from monohydric aliphatic saturated or unsaturated alcohols having from one through 18 carbon atoms and includes oleyl alcohol.

Mixed esters containing 75 mole per cent hydroabietyl 25 mole per cent oleyl ester may be made in any of the following or other suitable procedures.

A. Hydroabietyl alcohol (about 1.5 moles), oleyl alcohol (about 0.5 mole) and alpha-hydroxy aliphatic polycarboxylic acid (about 1.0 mole) are reacted as described hereinbefore.

B. About 75 mole parts of di-hydroabietyl ester of an alpha-hydroxy aliphatic polycarboxylic acid and about 25 mole parts of di-oleyl ester of an alpha-hydroxy aliphatic polycarboxylic acid are heated together until ester exchange has occurred.

C. Equal parts of 85 mole per cent hydroabietyl-15 mole per cent oleyl ester of an al-

pha-hydroxy aliphatic polycarboxylic acid and of 65 mole per cent hydroabietyl-35 mole per cent oleyl ester of an alpha-hydroxy aliphatic polycarboxylic acid are heated together until ester exchange has occurred.

D. A mechanical mixture is made of anhydroabietyl ester of an alpha-hydroxy aliphatic polycarboxylic acid and an ester of an alpha-hydroxy aliphatic polycarboxylic acid and a monohydric aliphatic alcohol having 8 to 20 carbon atoms in the proportion to produce the desired viscosity and the mixture added to the oil to be fortified.

In the foregoing the amount of hydroabietyl alcohol employed is based upon the hydroxyl number of the available mixture containing the hydroabietyl alcohol. That is to say, one mole of alcohol is equivalent to 17 grams of hydroxyl radical.

It is to be noted that while the neutral esters are satisfactory for use in cutting oils it is preferred to use esters which are a mixture of neutral and partial esters for anti-rust agents. Therefore, it is preferred to use esters having a neutralization number of zero to 30 in cutting oils but esters having a minimum neutralization number of 10 in anti-rust oils, such as turbine oils.

Those skilled in the art will understand that when compounding base oils with the novel esters other additives such as antioxidants, pour depressants, stain inhibitors, etc. etc., may be added in addition to the novel ester. Accordingly, the present invention contemplates the addition of the novel esters to simple or compound mineral oils of lubricating grade in the proportion of about 90 to about 99 per cent by weight of base oil to about 10 to 1 per cent, preferably 0.1 to 2 per cent by weight of the novel ester. In other words, the present invention provides a novel composition of matter comprising a major proportion of a base oil and a minor proportion of the novel esters effective to inhibit rusting and to enhance the extreme pressure properties of the base oil. The base oil is a lubricating fraction of mineral oil, a conventional gear lubricant base, a cutting oil or a grease.

We claim:

1. A novel composition of matter comprising moderately sulphurized mineral oil containing about 0.9% active sulphur, 0-99 weight percent; chlorinated base containing about 42% chlorine, 0-15 weight percent; mineral oil 50-500' @ 100° F. SUV, 0-99 weight percent, and about 0.1 to 10 weight percent of an ester product of malic acid in which about 50-100 mole percent of the radicals attached to the carbonyl carbon atoms through oxygen is radicals of hydroabietyl alcohol and the balance is a radical of a monohydric aliphatic alcohol having 8-20 carbon atoms.

2. A novel composition of matter comprising sulphurized and chlorinated fatty oil containing about 5% sulphur and about 5% chlorine, 0.25 to about 15 weight percent; mineral oil, 50-500' @ 100° F. SUV, about 78 to about 99 weight percent; stain inhibitor, 0.1 to 10 weight percent of an ester product of malic acid in which about 50-100 mole percent of the radicals attached to the carbonyl carbon atoms through oxygen is radicals of hydroabietyl alcohol and the balance is a radical of a monohydric aliphatic alcohol having 8-20 carbon atoms.

3. A novel composition of matter consisting es-

sentially of a major proportion of a base oil of petroleum origin and a minor proportion about 0.1 to about 10 percent by weight of an ester product of malic acid in which about 50-100 mole percent of the radicals attached to the carbonyl carbon atoms through oxygen are radicals of hydroabietyl alcohol and the balance is a radical of a monohydric aliphatic alcohol having 8-20 carbon atoms.

4. A novel composition of matter consisting essentially of a major proportion of a base oil of petroleum origin and a minor proportion effective to increase the oiliness of said base oil of a mixture of hydrogenated rosin hydrocarbons and an ester product of malic acid in which about 50-100 mole percent of the radicals attached to the carbonyl carbon atoms through oxygen is radicals of hydroabietyl alcohol and the balance is a radical of a monohydric aliphatic alcohol having 8-20 carbon atoms.

5. A novel composition of matter comprising:

Component— Per cent weight  
 Moderately sulfurized mineral oil— 30-99  
 Chlorinated base containing about  
 42% chlorine —————— 0-7 25  
 Mineral oil, 50-500" @ 100° F. SUV— 0-62  
 Ester product of malic acid in which  
 about 50 to 100 mole per cent of the  
 radicals attached to the carbonyl  
 carbon atoms through oxygen is  
 radicals of hydroabietyl alcohol  
 and the balance is a radical of  
 monohydric aliphatic alcohol hav-  
 ing 8-20 carbon atoms— 0.25- 2

6. A novel composition of matter comprising:

Component— Per cent weight  
 Sulphurized-chlorinated fatty oil— 0.25-15  
 Mineral oil, 50-500" @ 100° F. SUV— 78-99  
 Stain inhibitor —————— 0- 2 40  
 Ester product of malic acid in which  
 about 50-100 mole per cent of the  
 radicals attached to the carbonyl  
 carbon atoms through oxygen is  
 radicals of hydroabietyl alcohol  
 and the balance is a radical of a  
 monohydric aliphatic alcohol hav-  
 ing 8-20 carbon atoms— 0.1 - 5

7. A novel composition of matter comprising:

Component— Per cent weight  
 Sulphurized-chlorinated fatty oil— 0.5 -4.0  
 Mineral oil, 50-500" @ 100° F. SUV— 95- 99  
 Stain inhibitor —————— 0.1 -0.5  
 Ester product of malic acid in which  
 about 50-100 mole per cent of the  
 radicals attached to the carbonyl  
 carbon atoms through oxygen is  
 radicals of hydroabietyl alcohol  
 and the balance is a radical of  
 monohydric aliphatic alcohol hav-  
 ing 8-20 carbon atoms— 0.25-0.5

15 8. A novel composition of matter consisting essentially of a base oil of petroleum origin and a minor proportion about 0.1 to about 10 weight per cent of a mixture of (1) a half ester of malic acid and hydroabietyl alcohol and (2) a half ester of malic acid and an aliphatic monohydric alcohol having 8-20 carbon atoms in the molecule.

20 9. A novel composition of matter consisting essentially of a base oil of petroleum origin and a minor proportion about 0.1 to about 10 weight per cent of a mixture of (1) a half ester of malic acid and hydroabietyl alcohol and (2) a half ester of malic acid and an aliphatic monohydric alcohol having 8-20 carbon atoms in the molecule, said mixture of said half esters having been heated until ester exchange occurs.

LESLIE C. BEARD, JR.  
 RALPH V. WHITE.

#### REFERENCES CITED

35 The following references are of record in the file of this patent:

#### UNITED STATES PATENTS

| Number    | Name    | Date           |
|-----------|---------|----------------|
| 2,142,989 | Barrett | Jan. 10, 1939  |
| 2,384,595 | Blair   | Sept. 11, 1945 |
| 2,397,332 | Amott   | Mar. 26, 1946  |
| 2,436,272 | Snyder  | Feb. 17, 1948  |
| 2,443,579 | Fuller  | June 15, 1948  |

#### OTHER REFERENCES

“New Products and Materials,” Chem. Eng., January 1948. Copy in Div. 50.

**Certificate of Correction**

Patent No. 2,564,634

August 14, 1951

LESLIE C. BEARD, JR., ET AL.

It is hereby certified that error appears in the printed specification of the above numbered patent requiring correction as follows:

Column 2, line 22, for "Dehydroabietyl alcohol" read *Dehydroabietyl alcohol*; same line, for "Dihydroabietyl alcodol" read *Dihydroabietyl alcohol*; column 7, in the heading to the table, columns 4 and 5 thereof, for

| Viscos-<br>ity At<br>130° F. | SUV<br>(sec.) At<br>210° F. | read | Viscosity SUV (sec.)  |
|------------------------------|-----------------------------|------|-----------------------|
|                              |                             |      | At 130° F. At 210° F. |

column 8, line 6, for "anhydro-" read *an hydro-*; and that the said Letters Patent should be read as corrected above, so that the same may conform to the record of the case in the Patent Office.

Signed and sealed this 1st day of January, A. D. 1952.

[SEAL]

**THOMAS F. MURPHY,**  
*Assistant Commissioner of Patents.*